

C. S. KATZ.

FILLED BANGKOK HAT AND PROCESS FOR MAKING SAME.

APPLICATION FILED JUNE 2, 1920.

1,391,546.

Patented Sept. 20, 1921.

Fig. 1.



Fig. 2.



Fig. 3.



Inventor

C. S. Katz,

By-  
Geo. F. Kimmel. Attorney

# UNITED STATES PATENT OFFICE.

CHARLES S. KATZ, OF ST. LOUIS, MISSOURI.

## FILLED BANGKOK HAT AND PROCESS FOR MAKING SAME.

1,391,546.

Specification of Letters Patent. Patented Sept. 20, 1921.

Application filed June 2, 1920. Serial No. 386,050.

To all whom it may concern:

Be it known that I, CHARLES S. KATZ, a citizen of the United States, residing at St. Louis, in the State of Missouri, have invented certain new and useful Improvements in a Filled Bangkok Hat and Process for Making Same, of which the following is a specification.

This invention relates to hats known as Bangkok hats which are constructed of a leaf somewhat similar to a palmetto leaf said hats being unbleached in their finished form, presenting a lightish brown appearance when completed. All attempts to fill such a hat have heretofore proven futile for the reason that the material from which the hat was made would turn the filler as though oiled and it would run off without having any effect whatever on the hat. Attempts made to produce a bleached hat of this character were unsuccessful for the reason that the hat when bleached presented an unattractive appearance and in addition was sponge-like in texture and absorbed moisture readily so that it would not retain its shape or stand up under weather conditions.

The object of this invention is to produce a filled Bangkok hat which will resist weather conditions, that is one which does not readily absorb moisture and will more effectively retain its shape under exposure to all kinds of weather than either a Panama or an unfilled Bangkok.

In the accompanying drawing:

Figure 1 represents a perspective view of a hat constructed in accordance with this invention;

Fig. 2 is an enlarged detail sectional view of an untreated Bangkok hat; and

Fig. 3 is a similar view of the completed treated hat.

It has been found that while an unbleached Bangkok hat cannot be filled the hat after being bleached may be filled and that when a suitable filler having the gen-

eral characteristics of a Panama or Toyo filler is applied to a bleached Bangkok hat that it will produce a hat attractive in appearance, lighter than a Panama, which has greater body than the ordinary unfilled Bangkok hat and which will resist weather conditions better than either a Panama or an ordinary Bangkok owing to the fact that the filled Bangkok hat does not readily absorb moisture and retains its shape when exposed to dampness.

Any suitable filler may be used such for instance as that described in Patent No. 1,315,605, granted to Charles S. Katz, September 9, 1919 and consisting of zinc oxide, four pounds, magnesium sulfate two pounds, sulfur eight pounds, alcohol one-quarter gallon, a gelatinous substance such as "Callo sizing" or gum tragacanth one gallon, formaldehyde in its commercial state one sixteenth of a pint and glycerin one pound. This solution is applied to the surface of the hat with a sponge and after drying the surface is rubbed off with a clean cloth leaving the interstices between the straw filled.

In Fig. 2 a detailed section of an untreated Bangkok hat is shown, the fiber shown at 1 being in its natural state while in Fig. 3 a similar section is shown with the fiber 1<sup>a</sup> covered by the filler 2 having said filler arranged in the interstices between the fiber.

What is claimed is:

1. As an article of manufacture a bleached filled Bangkok hat.
2. A process of making a filled Bangkok hat which consists in first bleaching the hat and then applying a filler thereto.
3. A process of making a filled Bangkok hat which consists in first bleaching the hat and then applying thereto a filler having the general characteristics of a Panama or Toyo filler.

In testimony whereof I affix my signature hereto.

CHARLES S. KATZ.